

# UNITED STATES PATENT OFFICE.

CAROLINE J. M. BOHL, OF BROOKLYN, NEW YORK.

## MANUFACTURE OF MOLDS FOR CASTING METALS.

1,086,582.

Specification of Letters Patent.

Patented Feb. 10, 1914.

No Drawing.

Application filed May 1, 1913. Serial No. 764,891.

*To all whom it may concern:*

Be it known that I, CAROLINE J. M. BOHL, a citizen of the United States, and residing at Brooklyn, in the county of Kings and 5 State of New York, have invented certain new and useful Improvements in the Manufacture of Molds for Casting Metals, of which the following is a specification, such as will enable those skilled in the art to which 10 it appertains to make and use the same.

This invention relates to molds for casting metals, and the object thereof is to provide an improved mold for this purpose by means of which the delicate outlines and designs 15 of a finely wrought pattern can be perfectly reproduced in a mold from said pattern; a further object being to provide a mold for the purpose specified which will stand or resist the heat of a furnace and also the heat 20 of the metals poured into it without being fractured or broken.

In the practice of my invention I take equal quantities of plaster of Paris and ashes, which, being thoroughly ground or 25 pulverized and thoroughly mingled or reduced to a thick liquid of the consistency of cream by stirring thereinto and mingling therewith a requisite amount of water. In this operation there will be formed on the 30 surface of the liquid a greater or less amount of dirt or refuse matter which should be skimmed off. The liquid thus formed is poured over or around the desired pattern in a suitable receptacle to form the desired 35 mold; and after the liquid has been allowed to set or become hard, which operation takes about half an hour, the mold so formed is removed from the pattern, or the pattern from the mold. The mold is then slowly 40 dried in a low temperature of from 100 to 200° Fahrenheit, after which the mold is covered or painted with melted lard either on the inner side only, or on both the inner and outer sides according to the thickness of 45 the mold, after which said mold is put in an oven or furnace the temperature of which is gradually raised to from 800 to 1000° Fahrenheit, according to the thickness or mass of the mold, after which said mold is 50 allowed to cool. The plaster of Paris and ashes contain some objectionable or interfering substances which will be burnt out in the above operation, and this completes the mold which is now ready for use.

55 The above method of making a mold has an advantage over other and somewhat simi-

lar methods, in that the liquid composition consisting of plaster of Paris, ashes and water can be poured into a receptacle around a pattern instead of being pressed or rolled over or on the pattern, and by reason of this fact the molds can be made to great advantage especially when undercut patterns are used. A mold made in this manner will give a finer result in casting various metals 60 and especially brass which is one of the hardest metals to cast on account of the quantity of fumes or gases which it discharges in the operation of casting. The object of covering or painting the mold with 65 melted lard and then heating and drying it in an oven, as hereinbefore described, is to prevent the mold from absorbing moisture, and this renders my improved mold much 70 more efficient than others of this class especially, in the operation of casting brass, for which purpose no practical mold has heretofore been made, though many have claimed 75 to be able to do so. By means of my improved process a mold can also be made in 80 much less time than is ordinarily necessary, this process requiring but one or two hours, in some cases, in which other processes would require days. A mold made in this manner will also stand any metal or mixture of 85 metals, this result being also accomplished by reason of the extremely porous quality of the mold.

This invention is an improvement on that described and claimed in U. S. Letters Patent No. 924,728, dated June 15, 1909, and one of the objects of the process herein described and claimed, is to prevent the formation on the casting or product of a thin layer or coating of foreign or dirty substances which it is very difficult to remove, but which is entirely obviated by the improved process herein described.

The use of my improved process is not confined to the purpose or object herein set 100 out, as the same may be applied in making or manufacturing other articles or devices, and although I have described the use of lard for the purpose of painting the mold after it is formed and before drying or heating, it 105 will be apparent, that other oleaginous substances may be used.

Having fully described my invention what I claim as new and desire to secure by Letters Patent is:—

110 The method of making molds and other articles herein described, which consists of

mixing plaster of Paris and ashes and reducing the product by mingling water therewith to a thick liquid, pouring said liquid over or around a pattern in a suitable receptacle to form the mold, allowing the mold to set or become hard, separating the mold and pattern, slowly drying the mold in a low temperature of from 100 to 200° Fahrenheit, painting the mold with melted lard and 10 then heating said mold in an oven, gradu-

ally raising the temperature to from 800 to 1000° Fahrenheit.

In testimony that I claim the foregoing as my invention I have signed my name in presence of the subscribing witnesses this 15 29th day of April, 1913.

CAROLINE J. M. BOHL.

Witnesses:

C. MULREANY,  
S. ANDREWS.